

# UNITED STATES PATENT OFFICE.

WILLIAM E. JEANNOT, OF MUSKEGON, MICHIGAN, ASSIGNOR TO WEST MICHIGAN STEEL FOUNDRY CO., OF MUSKEGON, MICHIGAN, A CORPORATION OF MICHIGAN.

## CARBONIZING-BOX, ANNEALING-POT, AND SIMILAR ARTICLE.

1,380,804.

Specification of Letters Patent. Patented June 7, 1921.

No Drawing.

Application filed May 15, 1920. Serial No. 381,775.

To all whom it may concern:

Be it known that I, WILLIAM E. JEANNOT, a citizen of the United States, residing at Muskegon, in the county of Muskegon and 5 State of Michigan, have invented certain new and useful Improvements in Carbonizing-Boxes, Annealing-Pots, and Similar Articles, of which the following is a specification.

10 This invention relates to carbonizing boxes, annealing pots and similar receptacles composed of a ferrous alloy having a high melting point, and especial capacity to resist heat or oxidation, carbonization, 15 and changes in shape.

The chief object of the invention is to provide carbonizing boxes and the like, made of a relatively inexpensive alloy, so that they incorporate the above mentioned qualities to a marked degree.

20 The desired qualities are embodied in an alloy in accordance with my invention, by adding to iron or steel by any suitable process, silicon, carbon and manganese, and usually also phosphorus and sulfur, in suitable 25 proportions.

My experiments have shown that either iron or steel treated with silicon, with carbon and manganese in suitable proportions, 30 will become more and more heat resistant and cementation resistant as the silicon content is increased from 1% to 3.5%. I have not made alloys higher than 3.5% silicon but my experience leads me to believe that 35 alloys up to 5% or 6% will possess the same qualities.

The following table shows variations of the ingredients which will produce the above qualities:

40 Carbon..... .10 to .50  
Silicon..... 1.50 to 3.50  
Manganese..... .2 to .6  
Phosphorus under..... .04  
Sulfur under..... .04

45 The following table shows a wider range of variation of certain of the ingredients which will give desirable results in certain cases:

50 Carbon..... .0 to .50  
Silicon..... 1.0 to 6.00  
Manganese..... .10 to .8  
Phosphorus under..... .04  
Sulfur under..... .04

55 I have found that the following formula,

with more restricted ranges of silicon, manganese and carbon produces a carbonizing box or like receptacle having, to a marked degree, the qualities of resistance to heat, warping, oxidation, carbonization and cementation:

|                  |             |
|------------------|-------------|
| Silicon          | 2.5 to 3. % |
| Manganese        | .2 to .6 %  |
| Carbon           | .1 to .2 %  |
| Phosphorus under | .04% 65     |
| Sulfur under     | .04%        |

The most important element of the alloy for the present purpose is silicon. The element of second importance is manganese. 70 The element of third importance is carbon. The phosphorus and sulfur are of small importance except from a standpoint of molding. The percentage of these elements is kept low to prevent checking of the cast- 75 ings.

The action of the alloying ingredients in producing the desired result cannot be completely accounted for in the present knowledge of the art. 80

I have, however, demonstrated after study and experiment, by thorough tests under working conditions, that alloys composed as stated will embody the desired qualities to a marked degree. 85

Carbonizing boxes composed of a steel alloy produced within the range of the above formulas have a very high melting point, approximately 2600° F., are also highly resistant to oxidation in the presence of an 90 oxidizing flame, and are also highly resistant to carbonization or cementation; that is they will absorb carbon very slowly in comparison with steels of other composition when in the presence of carbonizing material. 95

Therefore, although the alloy is valuable for many purposes where the above qualities are desired, it is especially valuable for carbonizing pots, cyanid pots and the like in 100 which metal articles are placed with carbonizing material and subjected to intense heat in furnaces, and for melting pots for aluminum and other metals having a lower melting point than that of the metal container. 105

Metallic containers of this class when made of ordinary metal or alloys, have rather low critical points and are consequently more susceptible to warping or distortion, and at 110

the same time absorb the carbonizing material which they contain, and they also are readily oxidized by contact with the flame and oxygen of the furnace. The principal 5 effect of this oxidation is to render the boxes porous so that they are either entirely ruined in a relatively small number of heats, or waste a large part of the carbonizing material, which must be gasified for the pur-

10 pose of combining with the articles which are being treated; and if use of these defective boxes is continued they must be retained in the furnace for a longer time in order to properly treat the metallic contents.

15 The silicon content of the alloy renders the metal very homogeneous and sound, that is free from blow holes or gas occlusions. It also resists warping to a remarkable extent, even after a very large number of heats.

20 Certain alloys have been proposed for carbonizing boxes and the like which as a rule, depended upon a relatively expensive ingredient, such as nickel, to impart the desired qualities to the alloy. The most significant content of my alloy, as above stated, 25 is silicon, which is relatively inexpensive, and I am able to produce carbonizing boxes and other articles which are equal, if not superior, to any other alloys in the qualities 30 named, at a much lower cost.

An increase in the silicon content within reasonable limits, as suggested in the preceding formulas, increases the resistance of the alloy to heat and to carbonization, or 35 cementation. A decrease in the manganese content within reasonable limits, as above suggested, increases the resistance of the alloy to cementation. Decrease in the carbon content within reasonable limits raises 40 the melting point of the alloy.

So far as I am informed no alloy of similar composition has been suggested for carbonizing boxes and like articles; therefore 45 while silicon, carbon and manganese are frequently ingredients in ferrous alloys they have not been employed in a combination equivalent to the present one, or in such a way as to produce the desired results.

This application is a continuation in part 50 of my previous application Serial Number 340,443, filed November 25, 1919, including the subject matter of that application, with the addition of a slightly increased range of manganese.

55 Having thus fully described my invention, what I claim is:

1. A carbonizing box or like container

composed of ferrous alloy having as a leading ingredient silicon in proportion from 1 to 6%, together with carbon and manganese.

2. A carbonizing box or like container composed of a ferrous alloy having as a leading ingredient silicon in proportion from 1 to 6%, together with carbon, manganese, phosphorus and sulfur.

3. A carbonizing box or the like having a very high melting point and great resistance to oxidation and carbonization, consisting of a ferrous alloy including silicon 1 to 6%, manganese .10 to .8% and carbon .0 to .50%.

4. A carbonizing box or the like having a very high melting point and great resistance to oxidation and carbonization, consisting of a ferrous alloy including silicon 1.50 to 3.50%, manganese .30 to .8% and carbon .10 to .50%.

5. A carbonizing box or the like having a very high melting point and great resistance to oxidation and carbonization, consisting of a ferrous alloy including silicon 1 to 6%, manganese .10 to .8% and carbon .0 to .50%, phosphorus and sulfur each .04% or less.

6. A carbonizing box or the like having a very high melting point and great resistance to oxidation and carbonization, consisting of a ferrous alloy including silicon 1.50 to 3.50%, manganese .30 to .6% and carbon .10 to .50, phosphorus and sulfur each .04% or less.

7. A carbonizing box or like article adapted to contain articles for heat treatment at high temperature composed of a steel alloy having the following significant ingredients 95 in addition to the iron content; silicon 2.5 to 3.%, manganese .3 to .8%, carbon .1 to .2%, sulfur and phosphorus each .04% or less.

8. A carbonizing box or similar container 100 for treating articles at high temperature, highly-resistant to heat, oxidation and carbonization, composed of a silicon-alloy-steel, containing silicon in proportion from approximately 1. to 6%.

In testimony whereof I affix my signature in presence of two witnesses.

WILLIAM E. JEANNOT.

Witnesses:

JOHN Q. ROSS,  
ALICE WILSON.